

Patented Jan. 16, 1923.

1,442,631

# UNITED STATES PATENT OFFICE.

LAWRENCE GEORGE RICHARDSON, OF WEST BRIDGEFORD, NEAR NOTTINGHAM, ENGLAND, ASSIGNOR TO AMERICAN CELLULOSE AND CHEMICAL MANUFACTURING COMPANY LIMITED, OF NEW YORK, N. Y., A CORPORATION OF DELAWARE.

## TREATMENT OF PRODUCTS MADE WITH CELLULOSE DERIVATIVES.

No Drawing.

Application filed August 31, 1921. Serial No. 497,380.

To all whom it may concern:

Be it known that I, LAWRENCE GEORGE RICHARDSON, a subject of the King of Great Britain and Ireland, of West Bridgeford, 5 near Nottingham, England, formerly of Spondon, near Derby, England, have invented certain new and useful Improvements Relating to the Treatment of Products made with Cellulose Derivatives, of which the following is a specification.

In the process of preparing or dyeing of threads, filaments or fabrics of cellulose acetate, described in British Specification No. 11886 of 1920, and specification of United 15 States application Serial No. 461978, the cellulose acetate is subjected to a partial and limited degree of saponification before or during dyeing.

In those specifications the use of sodium 20 hydroxide was more particularly described as a matter of economy and convenience, it being understood that any other saponifying agents having a similar effect may be employed.

25 In carrying out the process originally described, it was found advantageous not to discharge the exhausted saponification bath after the treatment of the silk, but to use it again, repeatedly, after the addition each 30 time of the requisite fresh amount of sodium hydroxide solution, so that sodium acetate accumulated in the bath, and could ultimately be recovered.

It has been found that such accumulation 35 or presence of sodium acetate in the bath is of advantage not only from an economical point of view but also from a technical standpoint, as, amongst other facts, its presence in the bath intensifies or controls the 40 partial saponification and enables level dyeing to be more easily obtained on the goods.

According to the invention we add sodium acetate to the baths in which the partial 45 saponification of cellulose acetate threads, filaments or fabrics, and in particular of cellulose acetates lower than triacetate, is to be effected or it may be added to dyebaths when the partial saponification and dyeing 50 are conducted as a single operation in dyebaths which permit of the presence of sodium acetate.

The effect is not bound to any particular concentration of sodium acetate as it is obtained with very small amounts, e. g. solu-

tions of about 1% or with larger amounts or 55 with relatively high concentrations. The best effects are however found to be obtained with low concentrations of sodium acetate. The action of small quantities of sodium acetate in the bath is probably a 60 chemical one.

By way of example we may make up a fresh saponifying bath containing any convenient quantity of sodium acetate, for instance about 1 to 2%, say about 10 to 20 lb. 65 per 100 gallons, (though we do not confine ourselves to this amount as we may use more or less) and in this bath we may effect the partial saponification of 10 lb. of cellulose acetate silk after the addition of 0.25 to 0.5 70 lb. of sodium hydroxide at a temperature of about 50° to 75° C. until the sodium hydroxide is exhausted or approximately so. The exhausted bath may be repeatedly made up again with fresh quantities of sodium 75 hydroxide and used again for the treatment of fresh quantities of silk as before mentioned if so desired.

We do not bind ourselves to any definite concentration of added sodium acetate, nor 80 to any exact quantity of the sodium hydroxide or other saponifying agent, nor to the particular temperature indicated, for the partial saponification, but we state that the addition of quantities of sodium acetate, 85 preferably in small quantities, intensifies the reaction and favours the obtainment of level dyeing as mentioned above.

What I claim and desire to secure by Letters Patent is:—

1. The herein described method of facilitating the dyeing of threads, filaments or fabrics of or containing cellulose acetate, and in particular of cellulose acetates lower than triacetate, which comprises subjecting 95 the same to limited alkaline saponification in an aqueous bath containing sodium acetate.

2. The herein described method of facilitating the dyeing of threads, filaments or fabrics of or containing cellulose acetate, and 100 in particular of cellulose acetates lower than triacetate, which comprises subjecting the same to limited alkaline saponification in an aqueous bath containing a small quantity of sodium acetate.

3. The herein described method of facilitating the dyeing of threads, filaments or fabrics of or containing cellulose acetate,

and in particular of cellulose acetates lower than triacetate, which comprises subjecting the same to limited alkaline saponification in an aqueous bath containing about 1 to 2 5 per cent of sodium acetate.

4. The herein described method of facilitating the dyeing of cellulose acetate, and in particular of cellulose acetates lower than thiacetate, which comprises subjecting the 10 same to alkaline saponification in an aqueous bath containing sodium acetate and a quantity of alkaline saponifying agent sufficient only to effect partial saponification of the cellulose acetate, until the saponifying agent 15 is practically exhausted.

5. The herein described method of facilitating the dyeing of cellulose acetate, and in particular of cellulose acetates lower than triacetate, which comprises subjecting the 20 same to alkaline saponification in an aqueous bath containing sodium acetate and a quantity of caustic soda sufficient only to effect partial saponification of the cellulose acetate, until the caustic soda is practically 25 exhausted.

6. The herein described method of facilitating the dyeing of cellulose acetate, and in particular of cellulose acetates lower than triacetate, which comprises subjecting the 30 same to alkaline saponification in an aqueous bath at about 50°-75° C., containing sodium acetate and a quantity of alkaline saponifying agent sufficient only to effect partial saponification of the cellulose acetate, 35 until the saponifying agent is practically exhausted.

7. The herein described method of facilitating the dyeing of cellulose acetate, and in particular of cellulose acetates lower than triacetate, which comprises subjecting the 40 same to alkaline saponification in an aqueous bath, containing about  $\frac{1}{2}$  per cent sodium acetate and a quantity of alkaline saponifying agent sufficient only to effect partial saponification of the cellulose acetate, until the saponifying agent is practically 45 exhausted.

8. The herein described method of facil-

tating the dyeing of cellulose acetate, and in particular of cellulose acetates lower than triacetate, which comprises subjecting the same to alkaline saponification in an aqueous bath containing about  $\frac{1}{2}$  per cent sodium acetate and a quantity of caustic soda sufficient only to effect partial saponification of the cellulose acetate, until the caustic soda is practically exhausted.

9. The herein described method of facilitating the dyeing of cellulose acetate, and in particular of cellulose acetates lower than triacetate, which comprises subjecting the same to alkaline saponification in an aqueous bath at about 50°-75° C., containing about  $\frac{1}{2}$  per cent sodium acetate and a quantity of alkaline saponifying agent sufficient only to effect partial saponification of the cellulose acetate, until the saponifying agent is practically exhausted.

10. The herein described method of facilitating the dyeing of threads, filaments or fabrics of or containing cellulose acetate, and in particular of cellulose acetates lower than triacetate, which comprises subjecting the same to limited alkaline saponification in an aqueous dye bath containing sodium ace- 75

11. The herein described method of facilitating the dyeing of threads, filaments or fabrics of or containing cellulose acetate, and in particular of cellulose acetates lower than triacetate, which comprises subjecting the same to limited alkaline saponification in an aqueous dye bath containing a small quantity of sodium acetate.

12. The herein described method of facilitating the dyeing of threads, filaments or fabrics of or containing cellulose acetate and in particular of cellulose acetates lower than triacetate, which comprises subjecting the same to limited alkaline saponification in an aqueous dye bath containing about 1 to 2 90 per cent of sodium acetate.

In testimony whereof I have hereunto subscribed my name.

LAWRENCE GEORGE RICHARDSON.